

## UNITED STATES PATENT OFFICE

2,548,493

## ESTERS OF TRIMETHYLDIPIIC ACID

Richard F. Robey, Cranford, N. J., assignor to  
Standard Oil Development Company, a corpora-  
tion of Delaware

No Drawing. Application August 3, 1948,  
Serial No. 42,329

4 Claims. (Cl. 260—485)

1

This invention relates to a new class of compounds which have been found to be particularly suitable for use as synthetic lubricants because of their low pour points and high viscosity indices.

In the lubricant art, considerable progress has been realized in recent years in the production of lubricants characterized by one or more specific properties and adapted for particular uses. In the main, this progress can be attributed to two developments: the first, new refining procedures, and the second, addition agents capable of imparting particular properties to available lubricants. Thus, viscosity index improvers and pour depressants are added to automotive lubricants to render the lubricants more adaptable to wide changes in temperature conditions, while other agents are added to improve the load carrying properties of a lubricant which is to be employed, for example, under extreme pressure conditions.

Recently, in an effort to obtain superior lubricants endowed with specific and superior characteristics, a new field has been explored, namely, the synthesis of lubricants from various materials. Esters represent one class of materials which have attracted unusual interest as synthetic lubricants. In general, they are characterized by higher viscosity indices and lower pour points than mineral oils of corresponding viscosity. The esters described in the present specification have been found to exhibit these desirable characteristics. Lubricants possessing such properties are of special value in the lubrication of engines which are subjected to high temperatures such as combustion turbine engines, particularly those of the "prop-jet" type. Mineral oil lubricants containing added viscosity index improvers, thickeners or other highly non-volatile additives are undesirable for use in such engines because of the tendency to leave a residue which accumulates and interferes with the operation of the engine. A synthetic lubricant of the type described in the present specification is especially adapted to use under such conditions, since the lubricant contains no additives and thus tends to leave no residue upon volatilization.

It has been found that long chain esters of alkylated adipic acids are suitable for use as synthetic lubricants. These include esters of long chain alkylated adipic acids, e. g., octadecyl-adipic acid. A more preferred group of esters, notable especially for their high viscosity indices and low pour points, are the fully esterified trimethyladipic acids, wherein the esterifying group is an aliphatic hydrocarbon radical of 1

2

to 18 carbon atoms, chosen so that the total number of carbon atoms in both esterifying groups is 12 to 36. The esterifying groups may be saturated or unsaturated and may be of a straight chain or branched chain character. The groups which esterify the two carboxyl groups of the acid may be alike or unlike in chain length or other characteristics.

Trimethyladipic acid, which undoubtedly consists of a mixture of the two isomeric forms having the structures



and



20

may be readily prepared by oxidizing dihydroisophorone with nitric acid, a detailed method for carrying out the preparation being described hereinafter. The trimethyladipic acid may be readily esterified by refluxing with a suitable alcohol in the presence of a catalyst such as p-toluenesulfonic acid monohydrate and a suitable medium for entraining water during the reaction.

25

30

35

40

45

50

55

Aliphatic alcohols which are suitable for preparing the esters of the present invention include the primary alcohols, saturated and unsaturated, of the C<sub>2</sub> to C<sub>18</sub> range, e. g., methyl, ethyl, n-propyl, n-butyl, n-amyl, n-hexyl, n-octyl, n-decyl, n-dodecyl, n-tetradecyl, cetyl, oleyl and n-octadecyl alcohols, as well as branched chain primary alcohols, e. g., 2-ethylhexyl alcohol. Another group of alcohols especially adapted for use in connection with the present invention are the so called "Oxo" alcohols, prepared by the reaction of carbon monoxide and hydrogen upon C<sub>2</sub> to C<sub>17</sub> olefins obtainable from petroleum sources. Materials such as diisobutylene and polypropylene are suitable for this purpose. The alcohols obtained normally have a branched chain structure.

Data will be given below showing properties of a number of examples of esters of trimethyladipic acid, particularly with respect to their usefulness as synthetic lubricating oils. All of the esters were prepared by esterifying trimethyladipic acid, which was prepared by the following method: In an all-glass apparatus, consisting of a 3-liter flask fitted with a stirrer, condenser, and dropping funnel, was placed 1.5

liters (16 mols) of 50% aqueous nitric acid solution. This material was heated to boiling and 350 grams (2.5 mols) of dihydroisophorone was added dropwise at such a rate that refluxing continued rapidly. The refluxing was continued for several hours after the addition of the dihydroisophorone was complete. The resulting solution was nearly neutralized with sodium hydroxide, and the top layer resulting from this procedure was separated. After washing the product three or four times with a saturated aqueous sodium chloride solution, benzene was added and the water removed by azeotropic distillations. The solvent was then removed by vacuum stripping to give 307 grams of product. This material may be distilled or used in the crude state.

Each of the esters described in the table below was prepared by esterifying the trimethyladipic acid obtained in the above described process in accordance with the following procedure, which is perfectly general in its application: A mixture containing 1 mol of trimethyladipic acid, 2.2 mols of alcohol, 0.7% by weight of p-toluenesulfonic acid monohydrate, and a water entraining material such as benzene, toluene, naphtha, or the like, was refluxed until no more water collected in the water trap connected to the refluxing condenser. Then the mixture was washed three times with a saturated solution of sodium carbonate and once with water. After drying over a desiccant such as "Drierite" (anhydrous  $\text{CaSO}_4$ ), the product was stripped at 210-225° C. under 5 mm. pressure.

The esters obtained by the above typical reaction method were found to have the properties set forth in Table I.

35

Table I

| Alcohol Used in Esterification                            | Kinematic Viscosity |         | Viscosity Index | ASTM Slope | ASTM Pour Point | Cloud Point of Mixture of 25% Ester and 75% Mineral Oil <sup>1</sup> |
|-----------------------------------------------------------|---------------------|---------|-----------------|------------|-----------------|----------------------------------------------------------------------|
|                                                           | 100° F.             | 210° F. |                 |            |                 |                                                                      |
| C <sub>8</sub> "Oxo" alcohol from a C <sub>7</sub> olefin | 13.790              | 3.198   | 108             | 0.764      | °F.<br>-35      | °C.<br>-10                                                           |
| C <sub>8</sub> "Oxo" alcohol from diisobutylene           | 22.710              | 4.316   | 110             | 0.751      | °F.<br>-35      | °C.<br>-10                                                           |
| n-Decanol                                                 | 16.68               | 3.787   | 154             | 0.724      | °F.<br>-35      | °C.<br>-10                                                           |
| n-Dodecanol                                               | 21.420              | 4.752   | 158             | 0.674      | 5               | °C.<br>-10                                                           |

<sup>1</sup> A well refined, solvent-extracted paraffinic type lubricating oil of SAE-20 viscosity grade.

The above data indicate that the esters of trimethyladipic acid possess characteristics with regard to viscosity index and pour point which indicate their suitability for general use as lubricating oils.

In order to demonstrate the superiority as lubricating oils of esters of trimethyladipic acid, when compared with the corresponding esters of adipic acid and monomethyladipic acid, pour 60

55

point data for the n-dodecyl esters are given in Table II.

Table II

| 5  | Acid            | Alcohol     | ASTM Pour Point (°C.) |
|----|-----------------|-------------|-----------------------|
| 10 | Adipic          | n-Dodecanol | +36                   |
| 10 | α-Methyladipic  | do          | +16                   |
| 10 | β-Methyladipic  | do          | +10                   |
| 10 | Trimethyladipic | do          | -15                   |

The esters of the present invention not only possess good lubricating qualities in themselves but they may be also blended with mineral lubricating oils to give lubricants of improved viscosity index and pour point.

What is claimed is:

1. As a new composition of matter a fully esterified trimethyladipic acid, the esterifying radicals being alkyl radicals each containing 1 to 18 carbon atoms, the two esterifying radicals together containing a total of 12 to 36 carbon atoms.
2. A composition according to claim 1 in which the esterifying radicals are normal straight chain alkyl radicals of 10 to 12 carbon atoms each.
3. As a new composition of matter the di-n-dodecyl ester of trimethyladipic acid.
4. As a new composition of matter the di-n-dodecyl ester of trimethyladipic acid.

RICHARD F. ROBEY.

#### REFERENCES CITED

The following references are of record in the file of this patent:

#### UNITED STATES PATENTS

Number 2,448,259 Name Finch Date Aug. 31, 1948

#### OTHER REFERENCES

Beilstein: "Handbuch der organischen Chemie" (4th ed.), vol. 2, page 715 (1920), vol. 2, Second supplement, page 605.